

Feb. 4, 1958

R. N. HALL

2,822,309

P-N JUNCTION DEVICE AND METHOD OF MAKING  
THE SAME BY LOCAL FUSION

Filed June 20, 1955

Fig. 1.



Fig. 2.



Fig. 3.



Fig. 7.



Fig. 8.



Fig. 4.



Fig. 5.



Fig. 6.



Inventor:  
Robert N. Hall,  
by Paul A. Frank  
His Attorney.

# United States Patent Office

2,822,309

Patented Feb. 4, 1958

1

2,822,309

## P-N JUNCTION DEVICE AND METHOD OF MAKING THE SAME BY LOCAL FUSION

Robert N. Hall, Schenectady, N. Y., assignor to General Electric Company, a corporation of New York

Application June 20, 1955, Serial No. 516,637

14 Claims. (Cl. 148—1.5)

My invention relates to semiconductor devices of the P-N junction type and to a method of making the same. This application is a continuation-in-part of my copending application, Serial No. 415,875, filed March 12, 1954, which is a continuation-in-part of my application Serial No. 331,610, filed January 16, 1953, both of which are assigned to the present assignee, and now abandoned.

Semiconductors are materials whose electrical conductivity lies intermediate the poor conductivity of "insulators" and the good conductivity of metallic "conductors." Conduction in semiconductors is primarily electronic, the conduction carriers comprising either electrons or electron vacancies resulting from the movement of electrons. The degree of conductivity in such semiconductors is substantially affected by changes in temperature and by the amount and type of impurities found therein. Although the present invention may utilize various semiconductors, its chief advantages and widest commercial applications are realized when elemental semiconductors which have a diamond lattice crystal structure and which are found in group IV of the periodic table of elements, such as germanium or silicon, are employed.

These elemental semiconductors have become conventionally classified as either positive, P-type; negative, N-type; depending primarily upon the type and sign of their predominant conduction carriers. With P-type semiconductors, the direction of rectification as well as the polarity of thermoelectric, photoelectric, or Hall effect voltage are all opposite to that produced with N-type semiconductors. Conduction in N-type material is primarily by means of the movement of free electrons, while conduction in P-type material is primarily by means of the movement of "positive-holes" which arise from an electron vacancy in the electronic system of atoms of the material. It has been found that the determinant of whether a particular semiconductor body exhibits N-type or P-type characteristics lies primarily in the type of dominant impurity elements present in the semiconductor.

Some impurity elements, termed "donors," function to furnish additional free electrons to the semiconductor so as to produce an electronic excess material having N-type conductivity characteristics. Such material is denominated as N-type semiconductor. Other impurity elements, termed "acceptors," function to remove electrons from the semiconductor crystal lattice to create material with an excess of "positive-holes" having P-type conductivity characteristics. Such material is denominated as P-type semiconductor. Antimony, phosphorus, and arsenic, falling in group V of the periodic table, are examples of donor impurities in germanium and silicon, while aluminum, boron, gallium, and indium, falling in group III-B of the periodic table, are examples of acceptor impurities for germanium and silicon. True donors and acceptors such as those enumerated above are characterized in that they add or subtract respectively from the semiconductor lattice structure one electron per atom of impurity independent of temperature above such extremely low temperatures as

2

the boiling point of liquid air. Only very small amounts of these impurity elements are normally necessary to produce marked electrical characteristics of one type or the other. Concentrations of some impurities of less than one part per million may be sufficient.

P-N junction semiconductor units have a zone of P-type semiconductor adjoining a zone of N-type semiconductor to form an internal space charge barrier having a relatively large or broad area as distinguished from the point contact type of device. This junction possesses marked rectifying properties as well as thermoelectric and photoelectric properties. A semiconductor having a region of one conductivity type adjoining two regions of opposite conductivity type to form two P-N junctions can be used to make a three terminal amplifying device known as a transistor.

In the construction of such broad area or P-N junction devices, problems often arise because of their fragility and difficulty of assembly. In some types of devices this problem is minimized by first creating the junction within an ingot of monocrystalline semiconductor material and then cutting out portions of the ingot containing one or more P-N junctions for use as P-N junction devices. Such methods, however, require careful control of the process by which the activator impurities are selectively added to different portions of the semiconductor crystal.

It is, therefore, a primary object of my invention to provide an improved method which forms a P-N junction device from a monocrystalline semiconductor member by local fusion.

It is a further object of my invention to provide a local fusion method for making P-N junctions within a semiconductor body already containing distributed donor and acceptor activator elements therein.

Still another object of the invention is to provide a simple, reproducible method for producing two adjacent P-N junctions in a transistor-sized body of semiconductor material.

Still another object of the invention is to provide a simple method for reproducibly producing junction transistor devices.

Another object of the present invention is to provide an improved method for producing transistors having higher frequency ranges than heretofore available.

In accordance with my invention, a monocrystalline semiconductor body is prepared with both acceptor and donor activator elements therein in relative quantities so that one type of activator element predominates to give the semiconductor body initial overall characteristics of one conductivity type. The dominant activator is chosen to have a lower segregation coefficient than that of the other activator of the opposite type. This segregation coefficient is the ratio of the activator impurity per unit mass in solid phase to that per unit mass in the adjoining liquid phase portion in a growing crystal of semiconductor material. To form a junction within a semiconductor body so prepared, a portion of it is melted and then allowed to cool and recrystallize. Due to the difference in the segregation coefficients of the donor and acceptor activators, the recrystallizing portion rejects more of the dominant activator element having the low coefficient than it does of the other activator element so that the recrystallized portion assumes the conductivity characteristics corresponding to the type of conduction carriers produced by the activator element having the high segregation coefficient. Since the recrystallization starts or grows from the cooler portion of the melted semiconductor material adjacent the unmelted portion of the semiconductor body, a P-N junction between a zone of the original conductivity type and the converted opposite conductivity type is thus created.

In accordance with a further feature of the invention, the relative and absolute amounts of donor and acceptor impurities within the starting semiconductor ingot are chosen so as to take advantage of the fact that the segregation coefficients of certain impurity activators are strongly dependent upon growth rate. With the amounts of impurity activators so chosen, the melting and recrystallization is performed, as before, with the exception that the dependence of segregation coefficient upon growth rate causes a second reversal of conductivity-type semiconductor formed as the ingot recrystallizes. This second reversal of conductivity type results in a second P-N junction being formed in the growing ingot. The resultant ingot having therein two closely spaced P-N junctions is useful as a junction transistor.

The novel features which are believed characteristic of the invention are set forth in the appended claims. The invention itself, together with further objects and advantages therein, may best be understood by reference to the following description taken in connection with the accompanying drawing in which:

Figs. 1, 2 and 3 represent successive steps in preparing a P-N junction device in accordance with my invention; Fig. 4 is a group of curves illustrating the general variation of segregation coefficient with growth rate variation for certain exemplary acceptor and donor impurities; Fig. 5 is a graphical representation of the total segregation of selected impurity activators in germanium as a function of growth rate; Fig. 6 represents a semiconductive bar in which two P-N junctions are formed according to the invention; Fig. 7 represents an alternating embodiment of the device of Fig. 3, and Fig. 8 illustrates a junction transistor made in accordance with my invention.

Referring now to Fig. 1, a bar 1 of germanium is shown therein before the junction is formed. This bar contains both an acceptor impurity element and a donor impurity element uniformly distributed therein, one of the activator elements predominating so as to give the entire bar either P-type or N-type condition characteristics corresponding to the type of conduction carriers supplied by the dominant activator element. Such a bar may be extracted from a monocrystalline ingot grown by the seed crystal withdrawal method of Czochralski described, for example, in an article entitled "Preparation of germanium single crystals," by Roth and Taylor, in "The Proceedings of the IRE," vol. 40, pages 1338 to 1341, November 1952, or the "zone leveling" technique described, for example, in an article entitled "Principles of zone melting," by W. G. Pfann, on page 747, vol. 194, "Journal of Metals," July 1952. In the specific example indicated in Fig. 1, the dominant activator is indium, which, since it is an acceptor activator, furnishes positive conduction carriers or positive "holes" to give the germanium body P-type conductivity characteristics. The donor activator in this case is arsenic which, because it furnishes free electrons to the semiconductor body, would make it N-type except for the larger number of opposite-type conduction carriers supplied by the acceptor activator. While various activator elements may be selected, it is important that the dominant-type activator have a substantially lower segregation coefficient, which is the case in the example given since arsenic has a coefficient many times higher than that of indium. As previously stated, this segregation coefficient is defined as the ratio of impurity atoms per unit mass in solid phase to those in the adjoining material per unit mass in liquid phase in a growing crystal of semiconductor material. Thus, as a crystal of semiconductor material is grown from a melt of germanium containing traces of both high and low segregation coefficient activator elements, a relatively large percentage of the high coefficient element is assimilated in the growing crystal and a relatively small percentage of the low coefficient element is assimilated. For making junctions

in accordance with my invention, the semiconductor material of the bar 1 is prepared with the low segregation coefficient, dominant activator and the high segregation coefficient, opposite type of activator, both substantially uniformly dispersed or diffused within the semiconductor body. One method of preparing such material is described in greater detail in a subsequent paragraph.

As further shown in Fig. 1, one end, in this case the upper end, of the germanium bar 1 is heated until that end melts. Various means of heating or heat-treatment may be employed but it is essential that there be a temperature gradient in the germanium body 1 so that a portion of the germanium body is heated to a temperature high enough to produce fusion or melting while another portion remains below the melting point. Local fusion, such as produced by the flame of an oxyhydrogen torch 2 directed at one end of the bar-shaped germanium body 1, is illustrative of a simple way for producing such a gradient. Alternatively, local fusion may be caused by induction heating. The heating is preferably carried on in an atmosphere of nitrogen or other inert gas to prevent oxidation. The process may also be carried out within a vacuum, if desired, or in a reducing atmosphere.

After the heating, as indicated in Fig. 2, a portion 3 of the germanium body remains substantially unaffected by the heating process and retains its P-type characteristics. However, the melted portion which is allowed to recrystallize acquires N-type characteristics because the acceptor activator has been largely selectively rejected due to its low segregation coefficient, leaving the donor activator as the dominant activator element in that portion of the semiconductor body.

The melted portion 4 of the semiconductor body grows from the interface between the solid semiconductor of the lower portion 3 and the liquid semiconductor of the portion 4. The loss of heat from the melted portion to the solid portion is inherently greater than the loss to the surrounding atmosphere, and hence no special means are required to maintain the temperature differential required for directional cooling. Because of the surface tension of the molten material, the molten droplet of germanium remains in place without flowing away to become physically dissociated from the unmelted portion 3. However, due to the low segregation coefficient of the indium and due to the difference in segregation coefficients of the indium and the arsenic, a much greater proportion of the suspended arsenic than of the suspended indium is assimilated in the growing crystal. Thus, despite the preponderance of indium in the melted portion 4, the arsenic becomes the dominant activator element in the recrystallized portion and the rejected impurity elements within the portion 4 are increasingly concentrated in the still molten portion as the liquid-to-solid interface moves toward the upper end of the germanium bar 1.

Since the absolute values of the segregation coefficients for both arsenic and indium in germanium are both very small with respect to unity, the amount of arsenic and indium within the recrystallized portion 4 is much smaller than in the unmelted portion 3 of ingot 1. However, since the resistivity of both unmelted portion 3 and recrystallized portion 4 of ingot 1 depends, not upon the absolute amount of impurities present, but upon an excess of one type activator over the other type, the relative and absolute resistivities of regions 3 and 4 may be regulated and controlled merely by the selection of the relative and absolute amounts of donor and acceptor impurities in bar 1.

The transition plane at which the conductivity of the recrystallized portion becomes N-type constitutes a P-N junction between the two zones. This P-N junction possesses marked rectifying, photoelectric and thermoelectric effects. Since this P-N junction is located at the junction 75 between the fused and unfused portions of bar 8, it may

be readily located physically by the change in the shape of the bar due to fusion.

Referring now to Fig. 3, a completed P-N junction device 4 is shown in which electrical connections are made to the ends of the bar representing respectively the ends of the P-type and N-type zones, such as soldering conductors 7 thereto. The P-N junction semiconductor device so formed is a two-terminal device, suitable for uses such as electrical current rectification.

It is important that the activator elements and the relative quantities of each be properly selected in order that the semiconductor body for use in making P-N junctions in accordance with my invention can be correctly prepared. Reference is accordingly made to Fig. 4 which shows the variation with crystal growth rate of the segregation coefficients for donor activators antimony and arsenic and for acceptor activators gallium and indium in germanium. The growth rate increases when the temperature gradient within the liquid region is decreased in the process of growing a monocrystalline germanium ingot by withdrawing a seed crystal from a molten mass of germanium to which impurity elements have been added. The curves show that the segregation coefficients differ very widely and that the segregation coefficients of certain impurity activators increase as the growth rate increases.

Referring still to Fig. 4, it may be seen that if indium is to be employed as the acceptor activator and arsenic as the donor activator, that at any growth rate the proportion of the total arsenic in the melt assimilated in the growing crystal is many times greater than the proportion of the total indium in the melt assimilated in the growing crystal. Therefore, to obtain the preponderance of indium necessary to give the grown crystal overall P-type conduction characteristics, many times more indium than arsenic must be supplied to the melt. Thus, because each atom of arsenic donor element supplies one electron, and each atom of indium acceptor supplies one "hole" or positive carrier, the ratio of indium to arsenic by weight in the grown crystal must be greater than the ratio of their respective atomic weights. Since the segregation coefficient of arsenic in germanium is approximately 50 or more times that of indium, the atomic weight ratio in the melt must be increased by more than that factor. This principle governs as well when the invention is practiced with other donor and acceptor activators.

In Table I below, there are listed the equilibrium segregation coefficients of various donor and acceptor activator impurities in germanium and silicon respectively.

TABLE I

Equilibrium segregation coefficients

|    | Ge     | Si     |
|----|--------|--------|
| B  | ~20    | 0.68   |
| Al | 0.1    | 0.016  |
| Ga | 0.1    | 0.004  |
| In | 0.0011 | 0.0003 |
| P  | 0.12   | 0.04   |
| As | 0.04   | 0.07   |
| Sb | 0.004  | 0.018  |

Referring to Table I and to the description of the invention set forth hereinbefore, it is evident that a P-N junction may be formed in a semiconductor bar with any combination of donor and acceptor impurities having substantially different segregation coefficients. Thus, all combinations of any one of the acceptor activators, boron, aluminum, gallium, and indium in proper proportions with any one of the donor activators, will, in either germanium or silicon, produce a P-N junction by local fusion. The practical exceptions to this are combinations of phosphorus with either aluminum or gallium in germanium. Although junctions may be made, the closeness of the segregation coefficient of the donor phosphorus to the segregation coefficients of the acceptors gallium and

aluminum make extremely close control necessary. Other combinations having greater differences in segregation coefficients are preferred. In using any chosen donor-acceptor pair to practice the invention, it is only necessary that the activator having the lower segregation coefficient be in molar excess in the original bar.

The limits between which the relative amounts of selected donor and acceptor impurities added to a semiconductor melt from which a monocrystalline ingot is formed to produce semiconductor bars within which P-N junctions are formed by local fusion are as follows:

(1) In one limiting case, the low segregation coefficient, dominant impurity activator within the monocrystalline bar before fusion is exactly electrically compensated by the high segregation coefficient impurity activator.

(2) In the other limiting case, the high segregation coefficient activator impurity in the recrystallized portion of the ingot, after fusion, is exactly electrically compensated by the low segregation coefficient impurity.

Between these two limiting cases, all relative proportions of the selected donor and acceptor activator impurities will produce, after fusion, an ingot having a first region having the conductivity characteristics of the low segregation coefficient impurity, and a second region (the recrystallized region) having the conductivity characteristics of the high segregation coefficient impurity. These two regions are, of course, separated by a P-N junction.

The first limiting condition is expressed mathematically by the expression

$$\frac{Wt._a}{Mol\ wt._a} K_a \geq \frac{Wt._d}{Mol\ wt._d} K_d \quad 1(a)$$

where  $K$  is the segregation coefficient; the subscript  $(a)$  refers to acceptor impurity; the subscript  $(d)$  refers to donor impurity. This relationship applies to the case when the acceptor impurity is initially dominant and has a lower segregation coefficient than the donor impurity as, for example, when the impurities used are indium and arsenic. In this case the relationship states that the number of atoms of acceptor activator which are present in the once-processed bar before local fusion are equal to or greater than the number of atoms of donor activator.

The converse limiting case, when the donor activator impurity is dominant in the unfused bar and has the lower segregation coefficient, as, for instance, when the chosen activators are antimony and gallium, is given by the relationship:

$$\frac{Wt._d}{Mol\ wt._d} K_d \geq \frac{Wt._a}{Mol\ wt._a} K_a \quad 1(b)$$

The second limiting condition is expressed, in the case when the acceptor impurity has the lower segregation coefficient by the expression:

$$\frac{Wt._d}{Mol\ wt._d} (K_d)^2 \geq \frac{Wt._a}{Mol\ wt._a} (K_a)^2 \quad 2(a)$$

This expression means that the number of atoms of donor impurity entering the recrystallized portion of the bar is equal to or greater than the number of acceptor impurity atoms entering that portion. The converse limiting case, when the donor activator has the lower segregation coefficient, is given by the expression:

$$\frac{Wt._a}{Mol\ wt._a} (K_a)^2 \geq \frac{Wt._d}{Mol\ wt._d} (K_d)^2 \quad 2(b)$$

Combining Equations 1 and 2 above, the criteria for determining the limits within which the relative amounts of donor and acceptor activator impurities may be added to the original melt may be expressed as:

$$\frac{Mol\ wt._d}{Mol\ wt._a} \times \frac{K_a}{K_d} > \frac{Wt._d}{Wt._a} > \frac{Mol\ wt._d}{Mol\ wt._a} \times \left( \frac{K_a}{K_d} \right)^2 \quad 3(a)$$

7 where the acceptor has the lower segregation coefficient, and

$$\frac{\text{Mol wt.}_a}{\text{Mol wt.}_d} \times \frac{K_d}{K_a} > \frac{\text{Wt.}_a}{\text{Wt.}_d} > \frac{\text{Mol wt.}_a}{\text{Mol wt.}_d} \times \left( \frac{K_d}{K_a} \right)^2 \quad 3(b)$$

where the donor has the lower segregation coefficient. In the above equations, the terms

$$\frac{\text{Wt.}_a}{\text{Wt.}_d} \text{ and } \frac{\text{Wt.}_d}{\text{Wt.}_a}$$

represent the relative weight proportions of donor and acceptor activator impurities which are operative in producing at least one P-N junction in a semiconductor bar by local fusion. It should be noted, however, that this ratio refers to the additions of impurity activators to the original melt from which the semiconductor ingot is produced. The ingot is then cut into small bars and local fusion practiced upon individual bars.

The absolute amounts of donor and acceptor activator impurities which may be used in practicing the invention are not critical and the method is operative from the smallest measurable additions up to the maximum solid solubilities of the various elements in germanium and silicon. The particular absolute amounts of activator impurities used is a matter of design consideration and is governed by the conductivities desired in the resultant P-N junction devices.

As a practical matter, however, it is desirable that the absolute values of donor and acceptor impurities be chosen within the limits which will cause the majority conduction carrier excess in the initial bar upon which local fusion is practiced, and the majority conduction carrier excess in the recrystallized semiconductor droplet to be within the range useful in electronic signal translating devices. The preferable ranges within which the selected activator impurities should be added to a melt from which the initial semiconductor bar upon which local fusion is practiced are governed by the following boundary conditions.

Firstly, the preferable minimum addition of each impurity should be at least as great as that amount as would cause, in the absence of other impurities, the initially grown, unmelted bar to have a carrier concentration of the order of  $10^{14}$  carriers per cubic centimeter of semiconductor, corresponding to a resistivity of approximately 50 ohm-centimeters.

Secondly, the preferable maximum addition of each impurity should be no greater than that amount which would cause, in the absence of other impurities, the useful portion of the fused and recrystallized portion of the semiconductor (excluding the extreme tip end thereof) to have a carrier concentration of the order of  $10^{17}$  carriers per cubic centimeter of semiconductor, corresponding to a resistivity of approximately 0.05 ohm-centimeter.

These preferable ranges are set forth in Table II below. Certain impurity activators, however, have segregation coefficients so low that additions of sufficient amounts thereof to a semiconductor melt to satisfy the second boundary condition, above, render the growth of satisfactory crystals extremely difficult. For these impurities, marked by an asterisk in Table II, the upper limit of the preferable range has been set at arbitrary values at which satisfactory crystals may readily be grown from the initial melt.

TABLE II  
Absolute values of additions of impurity activators

|     | To germanium (per 100 gm.) | To silicon (per 100 gm.) |
|-----|----------------------------|--------------------------|
| B.  | 0.001-1 $\mu$ gm.          | 0.34 $\mu$ gm.-5 mgm.    |
| Al. | 0.6 $\mu$ gm.-6 mgm.       | 360 $\mu$ gm.-20 gm.     |
| Ga. | 1.4 $\mu$ gm.-14 mgm.      | 370 $\mu$ gm.-20 gm.     |
| In* | 200 $\mu$ gm.-20 gm.       | 8 mgm.-20 gm.            |
| P.  | 0.26 $\mu$ gm.-2 mgm.      | 5.6 $\mu$ gm.-140 mg.    |
| As. | 1.8 $\mu$ gm.-50 mgm.      | 7.6 $\mu$ gm.-110 mg.    |
| Sb. | 40 $\mu$ gm.-13 gm.        | 484 $\mu$ gm.-27 gm.     |

8 These amounts, for the purposes of this application, are referred to as "activator quantities" of the several impurities.

It will be appreciated, however, that within these ranges, the impurities must be selected in relative proportions as set forth in Equations 3 above, so that the impurity having the lower segregation coefficient dominates the electrical characteristics of the initial semiconductor bar before local fusion.

- 10 In one specific example of the invention, a high back voltage P-N junction-type diode having a strongly P-type zone and weakly N-type zone is made by preparing a melt consisting of 63 grams of high purity germanium having less than  $10^{14}$  atoms of impurities per cubic centimeter thereof, corresponding to a resistivity of above 20 ohm-centimeters, 7.0 milligrams of indium and 14 micrograms of arsenic. A monocrystalline ingot was then grown during solidification of the melt by the well-known seed crystal withdrawal technique generally known as the Czochralski technique. The resulting solidified monocrystalline ingot is then sliced longitudinally by a diamond saw into wires a few inches long and about 0.030 inch wide and and thick. The tip of the wire first grown is then heated for about 5 seconds using the reducing portion of the 25 flame of an oxyhydrogen torch (adjusted to very small oxygen content) in order just barely to melt the tip. The heat is removed and the melted tip allowed to cool and recrystallize, thereby to form P-N junction 6 at the boundary of the unmelted zone 4. The wire is then cut about 0.050 inch below the junction 6 to provide the P-N junction unit of Fig. 2. Nickel leads 7 are then soldered with a conventional tin alloy solder 13 to the opposite ends of this P-N junction unit at about  $250^{\circ}$  C. to form the diode of Fig. 3. Referring to Table I above, it will 30 be appreciated that such diodes having an initially P-type region and a recrystallized N-type region may also be formed by using other combinations of a low segregation coefficient acceptor and a higher segregation coefficient donor in proportions specified by Equation 3(a) above, and in activator quantities as specified in Table II above. Such other combinations are, for example, phosphorus-aluminum, phosphorus-gallium, and antimony-indium in germanium; also, phosphorus-aluminum, phosphorus-gallium, phosphorus-indium, and arsenic-aluminum, 35 arsenic-gallium, arsenic-indium, antimony-aluminum, antimony-gallium, and antimony-indium in silicon. Diodes of this type were found to pass a reverse leakage current of only about 0.2 milliampere at -100 volts while passing a forward current of about 14 milliamperes 40 at +1 volt.
- In another specific example of the invention, a high forward current diode having a strongly N-type zone and a weakly P-type zone is made by preparing a melt consisting of 20 grams of high purity germanium having less than  $10^{14}$  impurity atoms per cubic centimeter corresponding to a resistivity of above 20 ohm-centimeters, 150 milligrams of antimony and 0.5 milligram of gallium and then following the same procedures of crystal formation, local fusion, recrystallization and electrode connection set forth above in connection with the arsenic-indium impregnated germanium melt. The resulting diode, shown in Fig. 7, has reverse conductivity characteristics for corresponding zones of the diode shown in Fig. 3 and typically passes about 1 milliampere reverse current leakage 45 at -50 volts and about 50 milliamperes forward current at +1 volt. Referring to Table I above, it will be appreciated that such germanium diodes having an initially N-type region and a recrystallized P-type region may also be formed by using other combinations of a low segregation coefficient donor and a higher segregation coefficient acceptor in proportions specified by Equation 3(a) above, and in activator quantities as specified in Table II above. Such other combinations for germanium are, for example, boron-phosphorus, boron-arsenic, boron-50 antimony, aluminum-arsenic, and gallium-arsenic.

In yet another specific example of the invention, a high forward current diode was prepared by preparing a melt consisting of 27 grams of silicon having less than  $10^{14}$  impurity atoms per cubic centimeter thereof, which impurity corresponds to a resistivity in excess of 20 ohm-centimeters, 100 milligrams of chemically pure antimony, and 29.8 milligrams of a master alloy of the same high purity silicon as above, and 0.08% by weight of chemically pure boron, and then following the same procedures of crystal formation, local fusion, recrystallization and electrode connection as set forth in the previous examples. The resulting diode possessed characteristics similar to those of the other examples. Referring to Table I above, it will be appreciated that such silicon diodes having an initially N-type region and a recrystallized P-type region may also be formed by using other combinations of a low segregation coefficient donor and a higher segregation coefficient acceptor in proportions specified by Equation 3(a) above, and in activator quantities as specified in Table II above. Such other combinations for silicon are, for example, boron-phosphorus and boron-arsenic.

In growing the ingot or crystal of semiconductor to be subsequently employed for making P-N junctions by local fusion the temperature of the melt is kept constant as the growing crystal is withdrawn, or at least sufficiently constant so that the relative change in segregation coefficients of the arsenic and indium due to temperature change is not so great as to change the conductivity type of the growing crystal. In my copending patent application Serial No. 304,203, filed August 13, 1952, now abandoned, and assigned to the assignee of the present invention, a method of producing junctions by changing the rate of growth to thus utilize the relatively different activator segregation coefficient changes with temperature is disclosed and claimed. In the embodiment of the present invention described with relation to Figs. 1, 2 and 3, both in the preparation of a semiconductor ingot or crystal and in the subsequent preparation of a single P-N junction in the crystal, it is the difference in the segregation coefficient and not their relative changes with growth rate that produces the desired effect.

The dependence of segregation coefficients of certain activator impurities may, however, be utilized in producing semiconductor devices having therein two P-N junctions in accord with another feature of the present invention. In Fig. 5 of the drawing there is shown a graph of total segregation of selected activator impurities in germanium as a function of growth rate. The curves in the graph of Fig. 5 indicate the total amount of typical donor and acceptor impurities which enter into the growing recrystallized portion of a locally fused germanium bar and represent the product of segregation coefficient and the total available amount of impurities available to enter the growing crystal. The curves of Fig. 5 are specifically representative of segregation of antimony and gallium in germanium and may be derived from the curves for antimony and gallium of Fig. 4 by adjusting the total available amounts of antimony and gallium so that the product of available amounts and segregation coefficients causes the total segregation curves of antimony and gallium to intersect. When the total quantities of antimony and gallium in the original semiconductor bar are so chosen that the curves of total segregation versus growth rate intersect at a low growth rate, for instance, between 0 and 6 inches per hour, it is then possible to produce by local fusion a semiconductor ingot having therein two P-N junctions. Such a device may then be used as a transistor for the generation and amplification of electrical signals.

In Fig. 6 of the drawing, there is shown a semiconductor bar 8 including two P-N junctions formed in accord with this feature of the invention whereby the dependence of segregation coefficient of certain activator impurities upon growth rate is utilized. As is shown in Fig. 6, a bar of semiconductor material 8 of one conductivity type has a melted

and recrystallized portion 8a having a first zone 10 of opposite conductivity type and a second zone 11 of the original conductivity type. The device of Fig. 6 may be produced substantially as follows:

5 A bar 8 of a semiconductor, as, for example, germanium, may be cut from a crystal of germanium containing uniformly dispersed therein a donor activator impurity, the segregation coefficient of which is substantially dependent upon growth rate as, for example, antimony, and an acceptor activator impurity, the segregation coefficient of which is substantially independent of growth rate and higher in absolute value than the segregation coefficient of the chosen donor as, for example, gallium. The relative proportions of antimony and gallium are selected 10 according to criteria, more fully discussed hereinafter, so that the total segregation curves of antimony and gallium as shown in Fig. 5 of the drawing intersect at a low growth rate, for example, between 0 and 6 inches per hour. The relative proportions are such that the donor, antimony, is provided in sufficient quantity so that the original bar 8, before fusion, possesses N-type conductivity characteristics. The upper portion 8a of N-type germanium bar 8 is then caused to melt by a heating thereof, as, for example, with an oxyhydrogen torch as discussed with respect to Fig. 1 15 while the lower remaining part 9 remains in the solid state. The heating means is then removed and the fused portion 8a recrystallizes from the liquid-solid interface marking the junction between the lower unmelted portion 9 of bar 8 and the fused globule 8a. When the proportions of antimony and gallium have been so selected that the total segregation versus growth rate curves intersect as in Fig. 5 of the drawing, the first formed portion of the recrystallized globule 8a in the device of Fig. 5 possesses P-type 20 conductivity characteristics. This may readily be seen from the consideration of curve of Fig. 5 wherein it is seen that for slow growth rates, the total segregation of gallium is greater than the total segregation of antimony and a greater number of gallium atoms enters that portion of the crystal than do atoms of antimony, resulting in a 25 molar excess of acceptor (gallium) over donor (antimony) impurities and forming P-type germanium.

The predominance of gallium over antimony in the first recrystallized portion 10 of globule 8a is due to the fact that as the molten globule first begins to recrystallize, 30 growth progresses initially from zero growth rate, increasing as the globule 8a freezes. The growth rate is originally quite slow due to the fact that the rate of recrystallization of the globule depends upon the temperature gradient within the liquid region adjacent the liquid-solid interface, the growth rate being fastest for low gradients and slowest for high gradients. Since the temperature of the interface is always at the fusion temperature of the germanium-impurity alloy, and the temperature of the unmelted portion 9 of bar 8 does not vary substantially, the 35 temperature gradient across the interface depends primarily upon the maximum temperature within the melted globule 8a atop bar 8. When the recrystallized portion first begins to crystallize, the temperature of this globule is quite high and, accordingly, the original growth rate is 40 very slow. As recrystallization progresses, however, the temperature of globule 8a falls rapidly and the rate of growth of the recrystallized portion increases progressively, since as the temperature of the globule falls, the 45 growth rate increases. When the relative proportions of donor and acceptor activator impurities within bar 8 have been properly chosen so that the point at which the curves of Fig. 4 intersect is a growth rate very close to zero growth rate, preferably below 6 inches per hour, and globule 8a 50 cools at a rapid rate, only a very thin P-type region will have formed before the growth rate exceeds the critical value at which the curves intersect.

As further cooling takes place and the upper part 11 of the fused globule recrystallizes, the growth rate exceeds 55 the critical value and the remaining portion 11 of the re-

## 11

crystallized globule possesses N-type conductivity characteristics because a greater number of antimony atoms enter the growing crystal than atoms of gallium, causing a molar excess of donor (antimony) over acceptor (gallium) impurities within region 11. The intersection between the original N-type region 9 of ingot 8 and region 10 forms a P-N junction 6a and the boundary between P-type region 10 and recrystallized N-type region 11 forms a second P-N junction 6b.

Since it is necessary that the two P-N junctions of a junction transistor be located within a very close distance of one another, it is evident that the above-described change in growth rate to cause the formation of two closely spaced P-N junctions must be conducted at a very rapid rate. I have found that for the production of efficient junction transistors, the locally fused portion of bar 8 must be cooled at a rate greater than 10 centigrade degrees per second, and preferably of the order 100 to 500 centigrade degrees per second. If the fused portion of bar 8 is not cooled at a rate greater than 10 centigrade degrees per second, even if the relative amounts of donor and acceptor impurities are properly chosen, the two P-N junctions so formed will be separated by so great a distance that effective transistor action does not occur, particularly at high frequencies. According to the invention, rapid rates of cooling are assured by practicing local fusion upon individual transistor-sized bars. Such bars should have a maximum cross-sectional area of 15 square millimeters. Additionally, only a small portion of the semiconductor bar, approximately 0.1 to 50 cubic millimeters of semiconductor, is melted, thus insuring small thermal inertia and rapid cooling.

Thus, it may be seen that an N-P-N junction transistor is simply formed, the adjoining boundaries of the zones 9 and 10 and the zones 10 and 11 defining the P-N junction regions 6a and 6b, respectively. Connections are suitably made to the respective zones for transistor operation, the central zone being the base and the end zones 9 and 11 being the emitter and collector zones, respectively. The tip 12 of the upper zone 11 contains such a high concentration of residual activator elements that it serves chiefly as a conductive terminal.

While the particular combination of activator elements described is exemplary, other combinations may be employed so long as the low segregation coefficient activator which is dominant in unmelting bar 8 has a segregation coefficient that increases much faster with increasing growth rate than the opposite-type activator. This is because it is not possible to attain the near-balance condition of Fig. 5 and yet maintain the impurity with the growth-rate-sensitive segregation coefficient as the dominant impurity in original semiconductor bar 8. Thus, for example, since the donor elements arsenic, antimony and phosphorus all satisfy this condition in both germanium and silicon, referring to Table I, it may be seen that the invention may be practiced with the proper proportionate combinations in activator quantities of boron with arsenic, antimony or phosphorus. Such combinations are effective in either germanium or silicon. Additionally, the invention may be practiced with the combinations aluminum-antimony, aluminum-arsenic, gallium-antimony and gallium-arsenic, in germanium.

In order that this feature of the invention be practiced to form semiconductor units having two P-N junctions therein, the relative proportions of donor and acceptor activator impurities must be chosen so that the original bar 8, before local fusion, is dominated by the activator impurity having the segregation coefficient which is lower in absolute magnitude and which shows a substantial dependence upon growth rate. I have found from experiment that these criteria are satisfied when the weight ratio of donor to acceptor activator added to the melt from which bar 8 is formed varies between 0.5 and 1.0 times the ratio of their molecular weights times the square of

## 12

the inverted ratio of their segregation coefficients. This relationship may be expressed as

$$5 \quad 0.5 \frac{\text{Mol wt.}_d}{\text{Mol wt.}_a} \left( \frac{K_a}{K_d} \times \right)^2 < \frac{\text{Wt.}_d}{\text{Wt.}_a} < \frac{\text{Mol wt.}_d}{\text{Mol wt.}_a} \times \left( \frac{K_a}{K_d} \right)^2$$

Thus, for example weight ratios of antimony to gallium in germanium from 500 to 950 have been found to form N-P-N semiconductor units having two closely spaced P-N junctions therein defining a P-type layer from 0.0001 to 0.003 inch thick, which thicknesses are especially desirable in transistor devices. Satisfactory N-P-N units have also been formed using weight ratios of arsenic to gallium in germanium from 6.5 to 9.9. Likewise, useful N-P-N units have been formed using weight ratios of antimony to boron in silicon ranging approximately from 10,000 to 18,000.

The absolute amounts of donor and acceptor activator material which may be used in practicing this feature of the invention are governed by the same criteria and fall 20 within the same ranges set forth hereinbefore with respect to the hereinbefore discussed feature of the invention in which only one P-N junction is formed. The preferred ranges of absolute values of donor and acceptor which produce the most useful devices in practicing this feature 25 of the invention are set forth hereinbefore in Table II.

In a specific example of this feature of the invention, an N-P-N junction-type transistor shown in Fig. 8 having a desirably unusually thin P-type base layer 10a of the order of 0.001 inch thick is made by preparing a melt 30 consisting of 20 grams of high purity germanium containing less than  $10^{14}$  impurity atoms per cubic centimeter, and corresponding to a resistivity of greater than 20 ohm-centimeters, 150 milligrams of antimony and 0.20 milligram of gallium, and then following the same procedures 35 of crystal formation, local fusion, recrystallization and electrode connection set forth hereinbefore in connection with the arsenic-indium-impregnated melt. An additional electrode connection to thin P-type base layer 10a is made by connecting a lead 13 to the layer 10a by an 40 indium solder contact 14 is fused to and with the edge of layer 10a to make a good positive charge furnishing connection therewith. Fused indium contact 14 may be allowed to overlap P-N junctions 6a and 6b on either side of layer 10a since the indium is an acceptor activator and 45 converts the surface adjacent region to which it is fused into P-type material whereby a rectifying P-N junction connection is made between this indium-impregnated zone and the N-type zones 9 and 11 on either side of P-type layer 10a. This type of electrode connection to a thin 50 P-type layer of an N-P-N transistor forms a portion of the subject matter of Patent 2,705,767.

In yet another specific example of this feature of the invention, a melt was prepared containing 27 grams of silicon having less than  $10^{14}$  impurity atoms per cubic centimeter thereof, which purity corresponds to a resistivity in excess of 20 ohm-centimeters, 99 milligrams of chemically pure antimony and 29.8 milligrams of a master alloy of the same high purity silicon as above and 0.08% by weight of chemically pure boron. This master alloy was used in order to accurately control the very small amount of boron in the melt. The same procedure of crystal formation, local fusion, and recrystallization was followed to produce an N-type silicon bar approximately 0.060 inch long, approximately 0.030 inch wide and thick, 65 and having two P-N junctions therein defining a transverse P-type zone approximately 0.0005 inch thick. A low resistance base contact was made to this base zone by soldering an aluminum wire thereto at a temperature of approximately 600°C. Low resistance contacts were then made to the two opposed N-type zones by soldering thereto a wire of 99% gold and 1% by weight antimony at a temperature of approximately 450°C. The entire unit was then etched in a strong acid to remove surface impurities. The finished device was then useful as a high frequency transistor.

Transistors made in accord with the above-described methods may typically have a current gain factor from about 100 to 500 when used in a conventional grounded emitter amplifier circuit, and have very thin P-type layers about 0.001 inch thick. It will be appreciated that the thinner the P-type layer, the shorter the time of response of the transistor device to a change in excitation current. Such thin layers are produced because the rate of cooling during recrystallization is unusually rapid, for example, of the order of 150° C. per second and the ratio of the activators assimilated by the recrystallizing bar differs at a correspondingly rapid rate. If a substantial portion of the entire crystalline ingot grown during solidification from the melt is remelted and recrystallized without special provisions to convey heat away therefrom, the rate of cooling is slower, for example, of the order of 10° C. per minute, so that the various impurities are assimilated at a fairly constant ratio by the recrystallizing ingot so that only a P-N junction results at the border of the remelted region.

Thus, it may be seen that a very important feature of the invention is the attaining of very rapid cooling rates which naturally result from melting only a portion of a very small transistor-sized body of semiconductive material. The attainment of such rapid rates of cooling has two important results. Firstly, as is evident from the above, the very rapid cooling rates which result from the use of small units and partial melting thereof promotes variations in crystal growth rates. As is hereinbefore discussed, the using of the changing growth rates makes possible the formation of two P-N junctions in a semiconductor body which is small and which is only partially fused. If the body were large and no special provisions were made to convey heat away therefrom, or if, for some other reason, cooling did not occur rapidly, it would be impossible to form two closely adjacent P-N junctions which encompass an intermediate semiconductor region with sufficiently high conductivity as to form the base region of an efficient, operable transistor.

Secondly, the use of rapid cooling rates practically eliminates diffusion of impurity activator atoms from one zone to another and results in the formation of sharp, clearly defined P-N junctions which give improved rectification and signal translating characteristics to the devices so formed. As an example of these improved characteristics, transistors formed by local fusion typically have low frequency current amplification factors ( $\alpha_0$ ) as high as 0.997. Additionally, such transistors typically exhibit an  $\alpha$ -cutoff frequency in excess of 20 megacycles per second and oscillate at frequencies as high as 50 megacycles per second.

While the present invention has been described by reference to particular embodiments thereof, it will be understood that numerous modifications may be made by those skilled in the art without actually departing from the invention. I, therefore, aim in the appended claims to cover all such equivalent variations as come within the true spirit and scope of the foregoing disclosure.

What I claim as new and desire to secure by Letters Patent of the United States is:

1. A method of producing a junction transistor from a monocrystalline semiconductor body having conduction characteristics of one sign and containing dispersed therein a first activator element for producing dominant conduction carriers of said one sign and a second activator element for producing a lesser number of conduction carriers of the opposite sign, the equilibrium segregation coefficients of said activator element in said semiconductor each being less than unity said first activator element having a substantially lower segregation coefficient at a low crystal growth rate which increases relative to that of said second activator with increase in crystal growth rate, said first activator and said second activator impurities being present

within said body in a ratio of 0.5 to 1.0 times the ratio of their molecular weights times the inverted ratio of their segregation coefficients in said semiconductor which method comprises fusing only a portion of said semiconductor to produce a liquid-phase to solid-phase interface therein and allowing said fused portion to cool at a rate greater than 10 centigrade degrees per second and to rapidly recrystallize from said interface to form a first recrystallized zone grown at a relatively low growth rate having dominant conduction characteristics provided by said second activator element, and a second recrystallized zone grown at a relatively high growth rate having dominant conduction characteristics provided by said first activator element.

15 2. A method of producing a junction transistor which comprises forming a monocrystalline semiconductor body having conduction characteristics of one sign and containing dispersed therein a greater amount of a first activator element for producing conduction carriers of said one sign and a lesser amount of a second activator element for producing conduction carriers of the opposite sign, the equilibrium segregation coefficients of said activator elements in said semiconductor each being less than unity said first activator element having a substantially lower segregation coefficient at a low crystal growth rate which increases relative to that of said second activator with increase in crystal growth rate, said first activator and said second activator impurities being present within said body in a ratio of 0.5 to 1.0 times the ratio of their molecular weights times the inverted ratio of their segregation coefficients in said semiconductor fusing a portion of said semiconductor body to produce a liquid-phase to solid-phase interface therein, and allowing said fused portion to cool at a rate greater than 10 centigrade degrees per second and to rapidly recrystallize from said interface at successively increasing growth rates to form a first recrystallized zone grown at a relatively low growth rate having dominant conduction characteristics provided by said second activator element and a second recrystallized zone grown at a relatively high growth rate having dominant conduction characteristics provided by said first activator element.

30 3. A method of producing a junction transistor from a monocrystalline semiconductor body having conduction characteristics of one sign and containing dispersed therein a greater amount of a first activator element for producing conduction carriers of said one sign and a lesser amount of a second activator element for producing conduction carriers of the opposite sign, the equilibrium segregation coefficients of said activator elements in said semiconductor each being less than unity said first activator element having a substantially lower segregation coefficient at a low crystal growth rate which increases relative to that of said second activator with increase in crystal growth rate, said first activator and said second activator impurities being present within said body in a ratio of 0.5 to 1.0 times the ratio of their molecular weights times the inverted ratio of their segregation coefficients in said semiconductor which method comprises fusing a portion of said semiconductor body to produce a liquid-phase to solid-phase interface therein, cooling said fused portion at a rate greater than 10 centigrade degrees per second and recrystallizing said fused portion from said interface at successively increasing growth rates to form a first recrystallized zone grown at a relatively low growth rate having dominant conduction characteristics provided by said second activator element and a second recrystallized zone grown at a relatively high growth rate having dominant conduction characteristics provided by said first activator element.

35 4. A transistor made in accordance with the method of claim 3.

5. The method of producing an N-P-N junction semiconductor unit which method comprises preparing a melt consisting essentially of a high purity semiconductor, and activator quantities of an acceptor activator impurity and

a donor activator impurity, said donor activator impurity having a segregation coefficient in said semiconductor which is substantially lower than that of said acceptor activator, the equilibrium segregation coefficients of said activator elements in said semiconductor each being less than unity said donor and said acceptor activator impurities being present in relative proportions so that the weight ratio of the acceptor to donor activator is from 0.5 to 1.0 times the ratio of their molecular weights times the square of the inverted ratio of their segregation coefficients, growing a monocrystalline ingot having N-type conductivity characteristics from said melt, extracting a small crystal from said ingot, locally melting a surface adjacent region of the extracted crystal and allowing the melted portion of the crystal to recrystallize to form a first cool at a rate greater than 10 centigrade degrees per second and to rapidly recrystallized zone having P-type conductivity characteristics and a second recrystallized zone having N-type conductivity characteristics.

6. The method of producing an N-P-N junction transistor which method comprises preparing a melt consisting essentially of high purity silicon and an acceptor-donor activator impurities combination for silicon, said activator impurity combination being selected from the group consisting of boron-arsenic, boron-antimony, and boron-phosphorus, said donor and acceptor being added in activator quantities and in relative proportions so that the weight ratio of the selected acceptor to the selected donor is from 0.5 to 1.0 times the ratio of their molecular weights times the square of the inverted ratio of their segregation coefficients, growing a monocrystalline ingot having N-type conductivity characteristics from said melt, extracting a small crystal from said ingot, locally melting a surface adjacent region of the extracted crystal and allowing the melted portion of the crystal to cool at a rate greater than 10 centigrade degrees per second and to rapidly recrystallize to form a first recrystallized zone having P-type conductivity characteristics, and a second recrystallized zone having N-type conductivity characteristics.

7. The method of claim 6 in which the acceptor-donor combination is boron-antimony.

8. The method of producing an N-P-N junction transistor which method comprises preparing a melt consisting essentially of high purity germanium and an acceptor-donor activator impurity combination for germanium, said activator impurity combination being selected from the group consisting of aluminum-antimony, aluminum-arsenic, gallium-antimony, and gallium-arsenic, said acceptor and donor being added in activator quantities and in relative proportions so that the weight ratio of the selected acceptor to the selected donor is from 0.5 to 1.0 times the ratio of their molecular weights times the square of the inverted ratio of their segregation coefficients, growing a monocrystalline ingot from said melt, extracting a small crystal from said ingot, locally melting a surface adjacent region of the extracted crystal and allowing the melted portion of the crystal to cool at a rate of 100 to 500 centigrade degrees per second and to rapidly recrystallize to form a first recrystallized zone having P-type conductivity characteristics and a second recrystallized zone having N-type conductivity characteristics.

9. The method of claim 8 in which the acceptor-donor combination is gallium-antimony.

10. A semiconductor device comprising a monocrystalline semiconductor body having a first crystallized region having uniformly dispersed therein activator quantities of an impurity activator of a first conductivity inducing type, and an impurity activator of a second conductivity inducing type, the equilibrium segregation coefficients of said activator elements in said semiconductor each being less than unity said first type activator having a substantially lower segregation coefficient which increases substantially with increasing crystal growth rates, said first activator being present in molar excess over said second activator

to cause said first region to be of said first conductivity type, a second recrystallized region having uniformly dispersed therein said first and said second activator with said second activator present in molar excess over said first activator causing said second region to be of said second conductivity type and to form a P-N junction with said first region, a third recrystallized region having therein said first and second activator with said first activator present in molar excess over said first activator causing said third

10 region to be of said first conductivity type and to form a P-N junction with said second recrystallized region, and respective low resistance contacts to each of said regions.

11. An N-P-N junction transistor comprising a monocrystalline semiconductor body having a first crystallized region having uniformly dispersed therein activator quantities of an acceptor activator impurity and a molar excess of a donor activator impurity having a segregation coefficient lower than that of said acceptor impurity and which increases relative thereto with increasing crystal growth

20 rate to cause said first region to have N-type conductivity characteristics the equilibrium segregation coefficients of said activator elements in said semiconductor each being less than unity, a second recrystallized region having therein said donor impurity and a molar excess of said

25 acceptor impurity to cause said region to possess P-type conductivity characteristics and to form a P-N junction with said first region, a third recrystallized region having therein said acceptor activator impurity and a molar excess of said donor activator impurity to cause said region to exhibit N-type conductivity characteristics and to form a P-N junction with said second recrystallized region, and respective low resistance contacts to each of said regions.

12. The method of producing an N-P-N junction transistor, which method comprises preparing a melt consisting essentially of high purity germanium impregnated with antimony and gallium, said antimony and gallium being added to the melt in activator quantities and in relative proportions of 500 to 950 parts by weight of antimony to each part gallium, growing a monocrystalline

40 ingot having N-type conductivity characteristics from said melt, extracting a small crystal from said ingot, locally melting a surface adjacent region of the extracted crystal and allowing the melted portion of the crystal to cool at a rate greater than 10 centigrade degrees per second to rapidly recrystallize to form a first recrystallized zone having P-type conductivity characteristics and a second recrystallized zone having N-type conductivity characteristics.

13. The method of producing an N-P-N junction transistor which method comprises preparing a melt consisting essentially of high purity germanium impregnated with arsenic and gallium, said arsenic and gallium being added to the melt in activator quantities and in relative proportions of 6.5 to 9.9 parts by weight of arsenic to each part gallium, growing a monocrystalline ingot having N-type conductivity characteristics in said melt, extracting a small crystal from said ingot, locally melting a surface adjacent region of said extracted crystal and allowing the melted portion of the crystal to cool at a rate greater than 10 centigrade degrees per second to rapidly recrystallize to form a first recrystallized zone having P-type conductivity characteristics and a second recrystallized zone having N-type conductivity characteristics.

14. The method of producing an N-P-N junction transistor which method comprises preparing a melt consisting essentially of high purity silicon impregnated with antimony and boron, said antimony and boron being added in activator quantities and in relative proportions of 10,000 to 18,000 parts antimony to each part boron by weight, growing a monocrystalline ingot having N-type conductivity characteristics from said melt, extracting a small crystal from said ingot, locally melting a surface adjacent region of the extracted crystal and allowing the

60 melted portion of the crystal to cool at a rate greater than 10 centigrade degrees per second to rapidly recrystallize to form a first recrystallized zone having P-type conductivity characteristics and a second recrystallized zone having N-type conductivity characteristics.

15. The method of producing an N-P-N junction transistor which method comprises preparing a melt consisting essentially of high purity silicon impregnated with antimony and boron, said antimony and boron being added in activator quantities and in relative proportions of 10,000 to 18,000 parts antimony to each part boron by weight, growing a monocrystalline ingot having N-type conductivity characteristics from said melt, extracting a small crystal from said ingot, locally melting a surface adjacent region of the extracted crystal and allowing the

17

melted portion of the crystal to cool at a rate greater than 10 centigrade degrees per second and to rapidly recrystallize to form a first recrystallized zone having P-type conductivity characteristics and a second recrystallized zone having N-type conductivity characteristics.

References Cited in the file of this patent

## UNITED STATES PATENTS

2,567,970 Scaff et al. Sept. 18, 1951 10

18

2,583,008 Olsen Jan. 22, 1952  
 2,691,736 Haynes Oct. 12, 1954  
 2,739,088 Pfann Mar. 20, 1956

## FOREIGN PATENTS

510,303 Belgium Apr. 15, 1952

## OTHER REFERENCES

Pfann: Journal of Metals, July 1952, pages 747-753.